



US011272824B2

(12) **United States Patent**  
**Mukoyama**

(10) **Patent No.:** **US 11,272,824 B2**  
(b5) **Date of Patent:** **\*Mar. 15, 2022**

(54) **WATER-DISINTEGRABLE SHEET AND METHOD FOR MANUFACTURING WATER-DISINTEGRABLE SHEET**

(71) Applicant: **DAIO PAPER CORPORATION**, Shikokuchuo (JP)

(72) Inventor: **Shinpei Mukoyama**, Shikokuchuo (JP)

(73) Assignee: **DAIO PAPER CORPORATION**, Shikokuchuo (JP)

(\*) Notice: Subject to any disclaimer, the term of this patent is extended or adjusted under 35 U.S.C. 154(b) by 0 days.

This patent is subject to a terminal disclaimer.

(21) Appl. No.: **16/338,416**

(22) PCT Filed: **May 23, 2017**

(86) PCT No.: **PCT/JP2017/019158**

§ 371 (c)(1),  
(2) Date: **Mar. 29, 2019**

(87) PCT Pub. No.: **WO2018/061306**

PCT Pub. Date: **Apr. 5, 2018**

(65) **Prior Publication Data**

US 2019/0246863 A1 Aug. 15, 2019

(30) **Foreign Application Priority Data**

Sep. 30, 2016 (JP) ..... JP2016-193101

(51) **Int. Cl.**

**A47L 13/17** (2006.01)  
**A47K 10/16** (2006.01)

(Continued)

(52) **U.S. Cl.**

CPC ..... **A47L 13/17** (2013.01); **A47K 10/16** (2013.01); **D21H 11/18** (2013.01); **D21H 27/00** (2013.01); **D21H 27/005** (2013.01)

(58) **Field of Classification Search**

CPC ..... D21H 11/18; D21H 17/63; D21H 27/002; D21H 19/10; D21H 27/00; D21H 21/18;

(Continued)

(56) **References Cited**

U.S. PATENT DOCUMENTS

3,563,241 A \* 2/1971 Evans ..... A61L 15/28  
604/364

3,868,205 A 2/1975 Thomas  
(Continued)

FOREIGN PATENT DOCUMENTS

CN 1390997 A 1/2003  
CN 104271023 A 1/2015

(Continued)

OTHER PUBLICATIONS

Machine Translation of JP 11-206611-A (Year: 1999).\*

(Continued)

*Primary Examiner* — Jose A Fortuna

(74) *Attorney, Agent, or Firm* — Maier & Maier, PLLC

(57) **ABSTRACT**

A water-disintegrable sheet in which a base paper sheet is impregnated with an aqueous agent is provided. The base paper sheet has a weight per unit area of 30 to 150 gsm and includes a water-soluble binder and cellulose nanofibers. The aqueous agent includes a cross-linking agent which cross-links with a water-soluble binder. In the base paper sheet, content of the water-soluble binder and content of the cellulose nanofibers gradually increase from inside toward outside of the base paper sheet in a thickness direction. When a wear resistance test is performed three times using a Gakushin type fastness rubbing tester with a PP band as a rubbing finger and an average of measured values for the three times is calculated for each of a MD direction and a CD direction, each average value is at least 40.

**20 Claims, 11 Drawing Sheets**



|      |                                                   |                                     |                                          |             |
|------|---------------------------------------------------|-------------------------------------|------------------------------------------|-------------|
| (51) | <b>Int. Cl.</b>                                   |                                     | 2017/0160206 A1* 6/2017 Nuopponen .....  | C08L 1/00   |
|      | <b>D21H 27/00</b>                                 | (2006.01)                           | 2017/0306562 A1* 10/2017 Phipps .....    | D04H 3/08   |
|      | <b>D21H 11/18</b>                                 | (2006.01)                           | 2017/0314200 A1* 11/2017 Johansson ..... | C08J 9/28   |
| (58) | <b>Field of Classification Search</b>             |                                     | 2018/0098672 A1* 4/2018 Izumi .....      | B32B 29/005 |
|      | CPC .....                                         | D21H 27/30; D21H 17/06; D21H 17/43; | 2018/0146834 A1* 5/2018 Izumi .....      | D21H 27/30  |
|      |                                                   | D21H 19/00; A47L 13/17; A47K 10/16; | 2019/0003128 A1* 1/2019 Mukoyama .....   | B32B 3/263  |
|      |                                                   | A47K 2010/3266; B32B 2260/028       | 2019/0223680 A1* 7/2019 Yamazaki .....   | D21H 17/63  |
|      | See application file for complete search history. |                                     | 2019/0246863 A1* 8/2019 Mukoyama .....   | D21H 17/63  |
|      |                                                   |                                     | 2019/0276958 A1* 9/2019 Konishi .....    | D21H 13/08  |
|      |                                                   |                                     | 2021/0148053 A1* 5/2021 Yamazaki .....   | D21H 27/002 |

|                        |                         |                                   |
|------------------------|-------------------------|-----------------------------------|
| (56)                   | <b>References Cited</b> | FOREIGN PATENT DOCUMENTS          |
| U.S. PATENT DOCUMENTS  |                         |                                   |
| 10/2021 Yamazaki ..... |                         |                                   |
| 5,264,269 A            | 11/1993 Kakiuchi et al. | EP 0421163 A2 4/1991              |
| 5,281,306 A *          | 1/1994 Kakiuchi .....   | EP 0900878 A2 3/1999              |
|                        | C11D 17/041             | EP 1630288 A1 3/2006              |
|                        | 162/158                 | EP 3505038 A1* 7/2019 .....       |
| 6,106,928 A            | 8/2000 Laurent et al.   | EP 3521511 A1* 8/2019 .....       |
| 6,132,557 A            | 10/2000 Takeuchi et al. | EP 3533370 A1* 9/2019 .....       |
| 6,455,129 B1           | 9/2002 Kershaw et al.   | JP 61113896 A 5/1986              |
| 6,749,718 B2 *         | 6/2004 Takai .....      | JP 62126197 U 8/1987              |
|                        | D21H 25/005             | JP 02149237 A 6/1990              |
|                        | 162/115                 | JP 11206611 A * 8/1999            |
| 6,827,819 B2           | 12/2004 Dwiggins et al. | JP 3865506 B2 1/2007              |
| 9,399,841 B2 *         | 7/2016 Yamada .....     | JP 2007209657 A 8/2007            |
| 10,422,084 B2 *        | 9/2019 Mukoyama .....   | JP 2008094067 A 4/2008            |
| 11,155,966 B2 *        | 10/2021 Yamazaki .....  | JP 2009203412 A 9/2009            |
| 2003/0000665 A1 *      | 1/2003 Takai .....      | JP 2011030793 A 2/2011            |
|                        | D21H 25/005             | JP 5959695 B1 8/2016              |
|                        | 162/115                 | JP 6211160 B1 10/2017             |
| 2006/0037724 A1        | 2/2006 Akai et al.      | JP 6470236 B2 * 2/2019 .....      |
| 2007/0110963 A1        | 5/2007 Uehara et al.    | JP 6474923 B2 * 2/2019 .....      |
| 2007/0128411 A1        | 6/2007 Kawai et al.     | WO WO-2018037646 A1* 3/2018 ..... |
| 2008/0263797 A1        | 10/2008 Berger et al.   | WO WO-2018061306 A * 4/2018 ..... |
| 2009/0126885 A1        | 5/2009 Akai et al.      | D21H 13/17                        |
| 2010/0233481 A1 *      | 9/2010 Isogai .....     | D21H 11/18                        |
|                        | D21H 11/20              |                                   |
|                        | 428/401                 |                                   |
| 2011/0008638 A1 *      | 1/2011 Miyawaki .....   | JP 428/537.5                      |
|                        | D21H 11/18              |                                   |
| 2012/0246854 A1        | 10/2012 Uchiyama et al. |                                   |
| 2012/0277351 A1 *      | 11/2012 Yano .....      | D21D 1/34                         |
|                        | 524/35                  |                                   |
| 2013/0017349 A1 *      | 1/2013 Heiskanen .....  | C09D 10/12                        |
|                        | 428/36.1                |                                   |
| 2013/0209772 A1 *      | 8/2013 Sandstrom .....  | D21H 11/18                        |
|                        | 428/220                 |                                   |
| 2014/0182797 A1 *      | 7/2014 Paltakari .....  | D21H 17/24                        |
|                        | 162/72                  |                                   |
| 2015/0090414 A1 *      | 4/2015 Yamada .....     | B31D 1/0093                       |
|                        | 162/109                 |                                   |
| 2015/0167243 A1 *      | 6/2015 Bilodeau .....   | D21H 17/005                       |
|                        | 162/65                  |                                   |
| 2015/0267070 A1 *      | 9/2015 Tsuji .....      | C08L 1/02                         |
|                        | 106/163.01              |                                   |
| 2015/0315747 A1 *      | 11/2015 Heiskanen ..... | A47L 13/16                        |
|                        | 162/181.2               |                                   |
| 2016/0016717 A1 *      | 1/2016 Toubeau .....    | D21H 21/10                        |
|                        | 220/62.13               |                                   |
| 2016/0024718 A1 *      | 1/2016 Lee .....        | D21C 9/007                        |
|                        | 162/9                   |                                   |
| 2016/0053437 A1 *      | 2/2016 Husband .....    | D21H 5/1236                       |
|                        | 162/9                   |                                   |
| 2016/0168696 A1 *      | 6/2016 Missoum .....    | D21H 25/04                        |
|                        | 427/299                 |                                   |
| 2016/0355983 A1 *      | 12/2016 Yamada .....    | B31D 1/0093                       |
| 2017/0073893 A1 *      | 3/2017 Bilodeau .....   | D21D 1/306                        |

\* cited by examiner

## OTHER PUBLICATIONS

International Search Report (ISR) dated Jul. 4, 2017 issued in International Application No. PCT/JP2017/019158.

Japanese Office Action dated Jul. 4, 2017 issued in counterpart Japanese Application No. 2016-193101.

Japanese Office Action dated Nov. 14, 2017 issued in Japanese Application No. 2017-146973.

Japanese Office Action dated Oct. 16, 2018 issued in Japanese Application No. 2018-000955.

Written Opinion dated Jul. 4, 2017 issued in International Application No. PCT/JP2017/019158.

Office Action (Non-Final Rejection) dated May 12, 2020 issued in related U.S. Appl. No. 16/326,797.

Related U.S. Appl. No. 16/326,797; First Named Inventor: Kosuke Yamazaki; Title: "Water-Disintegrable Sheet and Method for Producing Water-Disintegrable Sheet"; Filed: Feb. 20, 2019.

Chinese Office Action (and English language translation thereof) dated Jul. 29, 2020 issued in Chinese Application No. 201780052138. 8.

"Chinese Office Action (and English language translation thereof) dated Mar. 11, 2021 issued in Chinese Application No. 201780060194. 6".

International Preliminary Report on Patentability (IPRP) dated Apr. 2, 2019 (and English translation thereof) in counterpart International Application No. PCT/JP2017/01915.

Extended European Search Report (EESR) dated Feb. 10, 2020 issued in European Application No. 17855265.9.

***FIG.1***

***FIG. 2A******FIG. 2B***

***FIG.3A******FIG.3B******FIG.3C***

***FIG.4A******FIG.4B***

***FIG.5***

**FIG. 6****FIG. 7****FIG. 8**

**FIG. 9****FIG. 10**

***FIG.11***

***FIG.12***

**FIG.13****FIG.14**

***FIG. 15A***



***FIG. 15B***



1

## WATER-DISINTEGRABLE SHEET AND METHOD FOR MANUFACTURING WATER-DISINTEGRABLE SHEET

### TECHNICAL FIELD

The present invention relates to a water-disintegrable sheet impregnated with an aqueous agent in advance, such as a toilet cleaning sheet, and a method for manufacturing the water-disintegrable sheet.

### BACKGROUND

Conventionally, there has been used a dust cloth for cleaning a toilet, which is made of woven fabric and can be used repeatedly. Instead, in recent years, a disposable water-disintegrable sheet made of paper is used.

This kind of water-disintegrable sheet is provided with a detergent impregnated, and can be processed by being flushed down the toilet after use.

Such a water-disintegrable sheet is required to have paper strength in a wet state impregnated with a detergent so as not to be torn during a wiping operation, and water-disintegrability so as not to clog piping when it is flushed down the toilet or the like. For effectively achieving these features, there is known a technique including usage of a water-disintegrable sheet to which a water soluble binder containing carboxymethyl cellulose (hereinafter referred to as CMC) is added as a base paper (refer to, for example, Japanese Patent No. 3865506).

### SUMMARY OF INVENTION

#### Technical Problem

A conventional water-disintegrable sheet is sometimes torn during cleaning of the toilet when it is used for rubbing the rim of a toilet bowl strongly, for example. However, when concentration of a CMC solution to be applied is increased in order to improve surface strength, the water-disintegrable sheet includes an increased amount of the CMC solution inside and thus has decreased water-disintegrability.

As described above, there has been a demand to improve tear resistance of a water-disintegrable sheet against strong rubbing while water-disintegrability is ensured.

The present invention has been made in view of the above problem, and an object of the present invention to provide a water-disintegrable sheet having improved tear resistance against strong rubbing while ensuring water-disintegrability, and a method for manufacturing the water-disintegrable sheet.

#### Solution To Problem

One aspect of the present invention is a water-disintegrable sheet in which a base paper sheet is impregnated with an aqueous agent. The base paper sheet has a weight per unit area of 30 to 150 gsm and includes a water-soluble binder and cellulose nanofibers, and the aqueous agent includes a cross-linking agent which cross-links with a water-soluble binder. In the base paper sheet, a content of the water-soluble binder and a content of the cellulose nanofibers gradually increase from inside toward outside of the base paper sheet in a thickness direction. In addition, when a wear resistance test is performed three times using a Gakushin type fastness rubbing tester with a PP band as a rubbing finger and an

2

average of measured values for the three times is calculated for each of a MD direction and a CD direction, each average value is at least 40.

Another aspect of the present invention is a method for manufacturing a water-disintegrable sheet. The method includes applying a water-soluble binder solution including a water-soluble binder and cellulose nanofibers to an outer surface of a base paper sheet, drying a sheet to which the solution has been added, and, after the drying, applying an aqueous agent including a cross-linking agent which cross-links with a water-soluble binder to the sheet. A concentration of the water-soluble binder solution is at least 3.3%, and a blending ratio of the water-soluble binder to the cellulose nanofibers in the water-soluble binder solution is 9:1 to 1:1.

The concentration of the solution can be at least 3.5%.

#### Advantageous Effects Of Invention

According to the present invention, it is possible to improve the tear resistance against strong rubbing, while ensuring the water-disintegrability. Therefore, the wiping property can be improved.

#### BRIEF DESCRIPTION OF DRAWINGS

FIG. 1 is a plan view showing an example of a toilet cleaning sheet according to the present embodiment.

FIG. 2A is a view showing fiber orientation of a conventional sheet.

FIG. 2B is a view showing fiber orientation according to the present invention.

FIG. 3A is an enlarged view and a sectional view of emboss portions of the toilet cleaning sheet.

FIG. 3B is an enlarged view and a sectional view of emboss portions of the toilet cleaning sheet.

FIG. 3C is an enlarged view and a sectional view of emboss portions of the toilet cleaning sheet.

FIG. 4A is an explanatory view showing an example of a contact area of the embosses.

FIG. 4B is an explanatory view showing an example of a contact area of the embosses.

FIG. 5 is a flowchart showing a method for manufacturing the toilet cleaning sheet according to the present embodiment.

FIG. 6 is a schematic view of equipment (solution addition equipment) for manufacturing the toilet cleaning sheet according to the present embodiment.

FIG. 7 is a schematic view of equipment (processing equipment) for manufacturing the toilet cleaning sheet according to the present embodiment.

FIG. 8 is a schematic view showing an example of a papermaking machine.

FIG. 9 is a graph showing evaluation of surface strength.

FIG. 10 is a graph showing evaluation of surface strength.

FIG. 11 is a graph showing evaluation of water-disintegrability.

FIG. 12 is a plan view showing another example of the toilet cleaning sheet according to the present embodiment.

FIG. 13 is a plan view showing another example of the toilet cleaning sheet according to the present embodiment.

FIG. 14 is an enlarged view of a portion A-A in FIG. 13.

FIG. 15A is an end view of a cut-off portion taken along line B-B in FIG. 14.

FIG. 15B is an end view of a cut-off portion taken along line C-C in FIG. 14.

#### DESCRIPTION OF EMBODIMENTS

Hereinafter, embodiments of the water-disintegrable sheet of the present invention are described in detail with refer-

ence to the drawings. However, the scope of the present invention is not limited to the illustrated examples.

The water-disintegrable sheet will be described using a toilet cleaning sheet as an example, but the water-disintegrable sheet also includes a wet tissue etc. impregnated with the aqueous agent for wiping other than a toilet cleaning sheet. The conveyance direction of the paper at the time of manufacturing the toilet cleaning sheet is referred to as the Y direction (length direction), and the direction orthogonal to the conveyance direction is described as the X direction (width direction).

[Description of Toilet Cleaning Sheet]

The toilet cleaning sheet **100** is formed by a ply process (lamination) of multiple (for example, two) base paper sheets and is impregnated with a predetermined aqueous agent. The base paper sheet may be formed of one base paper sheet to which the ply process has not been applied.

The weight per unit area of the base paper sheet is about 30 to 150 gsm. The weight per unit area is based on JIS P 8124.

The base paper sheet of the toilet cleaning sheet **100** is configured with a water-disintegrable fiber aggregate so that it can be discarded as it is in a toilet water pool after cleaning the toilet.

The fiber aggregate is not particularly limited as long as it has water-disintegrability, but a single layer or multiple layers of paper or nonwoven fabric can be suitably used. The raw material fiber may be a natural fiber or a synthetic fiber, and they may be mixed. Suitable raw material fibers include cellulosic fibers such as wood pulp, non-wood pulp, rayon, and cotton, biodegradable fibers made of polylactic acid, and the like. In addition, with these fibers as a main component, polyethylene fibers, polypropylene fibers, polyvinyl alcohol fibers, polyester fibers, polyacrylonitrile fibers, synthetic pulp, glass wool, and the like may be used in combination.

In particular, a fiber aggregate containing at least pulp is preferable, and suitable pulp used as a raw material includes leaf bleached kraft pulp (LBKP) and needle bleached kraft pulp (NBKP) blended at an appropriate ratio.

More preferably, a blending ratio of the leaf bleached kraft pulp exceeds 50% by weight. In other words, the blending ratio of the needle bleached kraft pulp to the leaf bleached kraft pulp is less than 1/1. As the blending ratio of the leaf bleached kraft pulp to the needle bleached kraft pulp is increased, gaps between fibers are reduced and moisture transpiration is suppressed. Therefore, it is possible to improve difficulty of drying.

Further, it may be configured of a sheet made of crushed pulp or a sheet of crushed pulp covered or sandwiched with water-disintegrable paper.

A water-soluble binder for enhancing paper strength is added to the base paper sheet of the toilet cleaning sheet **100**. Examples of the water-soluble binder include a binder component such as carboxymethyl cellulose, polyvinyl alcohol, starch or a derivative thereof, hydroxypropyl cellulose, sodium alginate, trant gum, guar gum, xanthan gum, gum arabic, carrageenan, galactomannan, gelatin, casein, albumin, purplan, polyethylene oxide, Viscose, polyvinyl ethyl ether, sodium polyacrylate, sodium polymethacrylate, polyacrylamide, hydroxylated derivatives of polyacrylic acid, polyvinyl pyrrolidone/vinyl pyrrolidone vinyl acetate copolymer, and the like.

In particular, from the viewpoint of good water-disintegrability and wet strength developed by cross-linking reaction, a water-soluble binder having a carboxyl group is preferably used.

The water-soluble binder having a carboxyl group is an anionic water-soluble binder which readily generates carboxylate in water. Examples thereof include polysaccharide derivatives, synthetic polymers, and natural products.

Examples of the polysaccharide derivative include a salt of carboxymethyl cellulose, carboxyethyl cellulose or a salt thereof, and carboxymethylated starch or a salt thereof, and an alkali metal salt of carboxymethyl cellulose (CMC) is particularly preferable.

CMC desirably has an etherification degree of 0.6 to 2.0, particularly 0.9 to 1.8, more preferably 1.0 to 1.5. It is because water-disintegrability and wet paper strength are excellently developed.

A water-swellable CMC is preferably used. This forms cross-links with a specific metal ion as the cross-linking agent in the aqueous agent and exerts a function of linking the fibers constituting the sheet while remaining unswollen. As a result, strength as a wiping sheet resistant to cleaning and wiping is exhibited.

In the case of the toilet cleaning sheet **100** of the present embodiment, CMC is added as the water-soluble binder.

Examples of the synthetic polymers include a salt of a polymer or a copolymer of an unsaturated carboxylic acid, a salt of a copolymer of an unsaturated carboxylic acid and a monomer copolymerizable with the unsaturated carboxylic acid, and the like. Examples of the unsaturated carboxylic acid include an acrylic acid, methacrylic acid, itaconic acid, crotonic acid, maleic anhydride, maleic acid, fumaric acid, and the like.

Examples of the monomer copolymerizable with them include an ester of the unsaturated carboxylic acid, vinyl acetate, ethylene, acrylamide, vinyl ether, and the like. A particularly preferred synthetic polymer is one using acrylic acid or methacrylic acid as the unsaturated carboxylic acid, and specifically include salts of polyacrylic acid, polymethacrylic acid, or acrylic acid methacrylic acid copolymer, and salts of a copolymer of acrylic acid or methacrylic acid, an alkyl acrylate or alkyl methacrylate. Examples of natural products include sodium alginate, xanthan gum, gellan gum, tarraganth gum, pectin, and the like.

Cellulose nanofibers (hereinafter referred to as CNF) are added to the water-soluble binder (CMC in the toilet cleaning sheet **100** according to the present embodiment).

A blending ratio of CMC to CNF is preferably 9:1 to 1:1. That is, in the water-soluble binder solution, CNF is included at least 10% by weight and at most 50% by weight. When the blending ratio is within this range, the surface strength of the toilet cleaning sheet **100** can be efficiently improved without increasing the amount of CMC.

Here, CNF refers to fine cellulose fibers obtained by fibrillating pulp fibers. In general, CNF refers to cellulose fibers containing cellulose fine fibers having a fiber width of nano-order size (at least 1 nm and at most 1000 nm). An average fiber width is preferably at most 100 nm. Number average, median, mode diameter (mode) and the like are calculated from a certain number of fibers and used as the average fiber width.

Examples of pulp fibers usable for manufacturing CNF include chemical pulp such as broad leaf tree pulp (LBKP) and needle leaf tree pulp (NBKP); mechanical pulp such as Bleaching thermomechanical pulp (BTMP), stone ground pulp (SGP), pressurized stone ground pulp (PGW), refiner ground pulp (RGP), chemi-ground pulp (CGP), thermogrind pulp (TGP), grand pulp (GP), thermomechanical pulp (TMP), chemi-Thermo Mechanical pulp (CTMP), and refiner mechanical pulp (RMP); used paper pulp manufactured from tea waste paper, craft envelope waste paper, magazine waste paper, newspaper waste paper, leaflets

waste paper, office waste paper, cardboard waste paper, high quality white waste paper, Kent waste paper, simili waste paper, regional waste paper, and groundwood paper; and deinked pulp (DIP) made by deinking used paper pulp. As long as the effects of the present invention are not impaired, these may be used alone or in combination of multiple kinds. Further, chemical treatment such as carboxymethylation may be applied to the pulp fibers before use.

Methods for manufacturing CNF are not limited to, but include mechanical methods such as a high pressure homogenizer method, a microfluidizer method, a grinder grinding method, a bead mill freeze pulverization method, and an ultrasonic fibrillating method. In addition, manufacture of nanofiber is promoted by using TEMPO oxidation treatment, phosphoric acid esterification treatment, acid treatment, etc. in combination.

The concentration of the water-soluble binder solution used for manufacturing the toilet cleaning sheet 100 of the present embodiment is at least 3.3% and at most 4.0%, preferably at least 3.5% and at most 4.0%, more preferably at least 3.8% and at most 4.0%. The application amount of the water-soluble binder solution to the base paper sheet is determined depending on the corresponding concentration so that the total amount of CMC-CNF attached to the base paper sheet after the application is constant.

When the concentration of the water-soluble binder solution is at least 3.3%, the surface strength of the toilet cleaning sheet 100 can be improved efficiently. The larger the concentration becomes, such as 3.5%, 3.8% etc., the more effects can be achieved. When the concentration is at most 4.0%, the toilet cleaning sheet 100 can be easily handled from the viewpoint of operation.

The viscosity of water-soluble binder solution is preferably at least 900 and at most 3000 centipoise (cP), when measured with a single-cylinder rotational viscometer (B-Type viscometer) under the condition of 60.degree. C. and 60 rpm.

In such a toilet cleaning sheet 100, the content of CMC-CNF in the raw paper sheet gradually increases from the inside toward the outside in the thickness direction. As a result, even if it is used for rubbing the rim of a toilet bowl strongly, the toilet cleaning sheet 100 is less likely to be torn than the conventional products uniformly impregnated with the water-soluble binder of the same amount.

A wear resistance test of the toilet cleaning sheet 100 was performed three times using a Gakushin type fastness rubbing tester with a PP band as a rubbing finger and an average of measured values for the three times is calculated for each of an MD direction and a CD direction, the average value was at least 40 for each direction.

In the above method of wear resistance test, the toilet cleaning sheet 100 was folded into three and the portion to be measured was rubbed with a Gakushin type fastness rubbing tester. The number of rubbing was obtained at the time when damage such as scuffing or tear was visually confirmed on the paper.

In the above wear resistance test, a PP band with a mesh pattern on the surface is used as the rubbing finger, assuming a case where the toilet cleaning sheet is actually used, that is, a case where the rim of a toilet bowl is rough due to attached stains. As a result, it is possible to conduct an environmental test assuming the actual use of the toilet cleaning sheet and to obtain highly reliable evaluation result on whether or not the toilet cleaning sheet is durable when actually used. If the measured value is at least 40 in the above wear resistance test, durability of the toilet cleaning sheet is considered to be sufficient in actual use.

The ratio (length/width) of fiber orientation in the length and width directions of the toilet cleaning sheet 100 is not particularly limited, but it is preferably 0.8 to 2.0, more preferably 0.8 to 1.2.

5 In the papermaking step which is a step for manufacture paper, as fibers are spread over wire(s) of a papermaking machine and flows in the transport direction, many fibers on the paper are generally aligned in the length direction, which is the conveyance direction by the papermaking machine 10 (for example, length:width=2.3:1; see FIG. 2A). Therefore, the fiber density in the width direction is low such that the fibers easily break. That is, the sheet is easily torn depending on the wiping direction. Therefore, in the present embodiment, as shown in FIG. 2B, the fiber orientation ratio in the 15 length and width directions of the toilet cleaning sheet 100 is set to be 0.8 to 2.0, preferably 0.8 to 1.2. As a result, it is possible to provide the toilet cleaning sheet 100 which is not easily torn even by wiping with the sheet in any direction. The fiber orientation ratio in the length and width directions 20 can be obtained from the ratio of a wet strength in the MD direction to that in the CD direction.

The toilet cleaning sheet 100 of the present embodiment is impregnated with a predetermined aqueous agent containing the cross-linking agent for cross-linking of the water-soluble binder, specifically, a predetermined aqueous agent containing, in addition to the cross-linking agent, an aqueous detergent, a fragrance, an antiseptic, a disinfectant, an organic solvent and the like, including an auxiliary agent. The aqueous agent for impregnation is 100 to 500% by 30 weight relative to the weight of the base paper sheet as the base material of the toilet cleaning sheet 100, preferably 150 to 300% by weight.

As the cross-linking agent, boric acid, various metal ions and the like can be used, but a polyvalent metal ion is 35 preferably used when CMC is used as the water-soluble binder. In particular, preferably used is one or more of polyvalent metal ions selected from the group consisting of alkaline earth metals, manganese, zinc, cobalt, and nickel, from the viewpoint of developing wet strength for durability in use by sufficiently bonding the fibers and from the viewpoint of improving water-disintegrability sufficiently. Among these metal ions, ions of calcium, strontium, barium, zinc, cobalt, or nickel are used particularly preferably.

As the aqueous detergent in addition to a surfactant, lower 40 or higher (aliphatic) alcohol may be used, for example.

As the fragrance, for example, one or several kinds of oily fragrance such as orange oil, in addition to an aqueous fragrance, may be appropriately selected and used.

As the antiseptic, for example, parabens such as methylparaben, ethylparaben, propylparaben, and the like may be used. As the disinfecting agent, for example, benzalkonium chloride, chlorhexidine gluconate, povidone iodine, ethanol, benzyl cetyl oxide, triclosan, chloroxylenol, isopropylmethylphenol, and the like may be used. As the organic solvent, 50 polyhydric alcohols such as glycol (divalent), glycerin (trivalent), sorbitol (tetravalent), and the like may be used.

Further, the auxiliary agent of the above-mentioned components of the aqueous agent may be selected appropriately, and a component which fulfills other functions may be 55 contained in the aqueous agent as necessary.

In this way, the water-soluble binder and cellulose nanofibers are blended into the base paper sheet and the sheet is 60 impregnated with the aqueous agent containing the cross-linking agent which cross-links with the water-soluble binder. Thus, the wet tensile strength can be improved according to the present invention as compared with the case where the base paper sheet into which the water-soluble

binder is blended is further impregnated with the aqueous agent containing the cross-linking agent which cross-links with the water-soluble binder.

The surface of the toilet cleaning sheet 100 may be the paper sheet as it is, but is preferably embossed. In the case of the toilet cleaning sheet 100, for example, two kinds of embosses EM11 and EM12 are made thereon, as shown in FIG. 1.

Although the shape, number, area ratio, etc. of the embosses are arbitrary, in the case of the toilet cleaning sheet 100, the embosses EM11 are arranged to form a diamond lattice. As a result, unevenness of wiping can be reduced as compared with the case where the embosses EM11 are arranged to form a square lattice or a rectangular lattice. The embosses EM12 are arranged between the embosses EM11.

Each of the embosses EM11 has, as shown in FIG. 3A, a protrusion PR21 having a curved shape.

Each of the embosses EM12 has, as shown in FIG. 3B, a protrusion PR22 having a plane shape.

Since the embosses EM12 are each arranged between the embosses EM11, the protrusions PR21 of the embosses EM11 and the protrusions PR22 of the embosses EM12 closely adheres to each other to form a continuous emboss EM21 as shown in FIG. 3C.

Alternatively, the protrusions PR21 of the embosses EM11 and the protrusions PR22 of the embosses EM12 do not have to be continuous but may be merely close to each other.

By forming the two kinds of embosses EM11 and EM12 in this way, it is possible to increase contact areas with the object to be cleaned. As a result, the toilet cleaning sheet 100 becomes less stiff and has higher wiping property.

That is, as a result of forming the embosses EM11 with the protrusion PR21 having a curved surface and the embosses EM12 with the protrusion PR22 having a plane surface on the entire sheet surface of the toilet cleaning sheet 100, the respective embosses are deformed for the first time when a force is applied to the toilet cleaning sheet 100 during the wiping operation so that the contact areas increase. Therefore, it is possible to improve flexibility due to deformation of the respective embosses, as well as to increase the contact areas.

For example, if there is a single kind of embosses EM11, the contact areas CN31 are formed discretely in the vicinity of the respective embosses EM11 after deformation of the embosses EM11 due to the force applied to the toilet cleaning sheet 100 during the wiping operation, as shown in FIG. 4A. On the other hand, if there are two kinds of embosses EM11 and EM12 in combination, as compared with the contact area CN31 of FIG. 4A, the contact areas SN32 become large after deformation of the embosses EM11 and EM12 due to the force applied to the toilet cleaning sheet 100 during the wiping operation as shown in FIG. 4B.

Further, the two kinds of embosses EM11 and EM12 also exhibit the effect of ordinary embosses, such as improvement of texture, absorbency, bulkiness, etc. of the toilet cleaning sheet. Furthermore, the continuous embosses EM21 also exhibit the effect of good appearance by embossing, as well as ordinary embosses.

The toilet cleaning sheet 100 is folded in two by a fold process at the center portion in the Y direction. Then, it is stored in a plastic case for storage or in a packaging film in a folded state, and unfolded as necessary at the time of use. The folding of the toilet cleaning sheet 100 is not limited to folding in two, but may be folding in four or eight, for example.

[Method for Manufacturing Toilet Cleaning Sheet]

Next, a method for manufacturing the toilet cleaning sheet will be described. FIG. 5 is a flowchart showing a method for manufacturing the toilet cleaning sheet. FIG. 6 is a schematic diagram of solution adding equipment for adding a water-soluble binder solution to the base paper sheet (paper sheet) of the toilet cleaning sheet. FIG. 7 is a schematic view of processing equipment for processing the base paper sheet to which the water-soluble binder solution has been added in the solution adding equipment shown in FIG. 6.

In the method for manufacturing the toilet cleaning sheet, as shown in FIG. 5, first, a papermaking step (S1) of making a paper to be a base paper (not shown) is performed with a papermaking machine.

Next, as shown in FIGS. 5 and 6, in the solution addition equipment, the ply processing step (S2) of making a ply continuous sheet 1B by the ply process of the continuous dry base paper 1A, 1A which are respectively drawn out from multiple (for example, two) primary web roll 1, 1 on which the base paper is wound up after papermaking; a solution adding step (S3) of adding the water-soluble binder solution to the ply continuous sheet 1B to form a continuous sheet 1C; a drying step (S4) of drying the continuous sheet 1C; and a slit-forming and winding step (S5) of forming a slit and winding the dried continuous water-disintegrable sheet 1D are performed. Although the number of primary web rolls can be appropriately changed as long as it is two or more, in the following descriptions, an example of using two primary web rolls will be described.

Next, as shown in FIGS. 5 and 7, in the processing equipment, an embossing step (S6) of embossing the continuous water-disintegrable sheet 1D drawn out from the secondary web roll 11 after winding in the slit-forming and winding step (S5), and a finishing step (S7) of applying a finish process to the embossed sheet 1E on which embossing has been performed.

Details of each step is described below.

[Papermaking Step]

First, the papermaking step (S1) according to the present embodiment will be described. In the papermaking step (S1) of the present invention, for example, the base paper sheet is formed by making a papermaking raw material by a known wet papermaking technique. That is, after making the papermaking raw material in a state of wet paper, it is dried with a dryer or the like to form the base paper sheet such as thin paper or crepe paper.

Besides pulp and a coagulant, papermaking chemicals such as wet paper strength agent, adhesive, release agent and the like may be appropriately used in the base paper sheet.

In addition, although the water-soluble binder solution is added in a solution addition step in the solution addition equipment described later in the embodiment of the present invention, the water-soluble binder solution may be added in the papermaking step.

If the water-soluble binder solution is also added in the papermaking step, it is possible to obtain a water-disintegrable sheet having large total strength. Then, by further adding the water-soluble binder solution in the subsequent step of the solution adding step, the surface strength of the water-disintegrable sheet can be further increased.

As a method of adding the water-soluble binder solution in a papermaking step, for example, a method of wet papermaking using a raw material in which the water-soluble binder and a fixing agent to fix the water-soluble binder to the pulp fibers are added to a dispersion containing pulp as a papermaking raw material (Japanese Unexamined

Patent Publication No. hei3-193996). That is, the water-soluble binder is internally adding in the method. It is also possible to perform wet papermaking of a sheet from a dispersion containing pulp, to spray and dry or to coat and dry the water-soluble binder after press dewatering or semi-drying, and to manufacture a fiber sheet containing a predetermined amount of the water-soluble binder. That is, the water-soluble binder is externally added in the method. In this case, it is possible to obtain a fiber sheet with a lower density and better water-disintegrability by using a pre-drying system such as a hot air passage dryer rather than press dewatering. Furthermore, instead of the wet papermaking method described above, it is also possible to manufacture a fiber sheet by fibrillating the dry pulp fibers without using water, forming a web, spraying the water-soluble binder, and then drying. It is a so-called air laid manufacturing method.

FIG. 8 shows a schematic diagram of an example of a manufacturing apparatus preferably used for manufacturing a fiber sheet where the water-soluble binder is used as a binder. The manufacturing apparatus (wet papermaking machine) shown in FIG. 8 is provided with a former 14, a wire part, a first dry part 17, a spray part, and a second dry part 24.

The former 14 adjusts the finished paper material supplied from a preparation device (not shown) to a predetermined concentration and then supplies it to the wire part. The preparation device (not shown) is provided with a device for separating and pulverizing raw materials such as pulp fibers and an adding device for adding additives such as a sizing agent, a pigment, a paper strengthening agent, a bleaching agent, a coagulant and the like to the separated and pulverized raw material, and is configured to prepare the paper material including a raw material at a predetermined concentration according to the features of water-disintegrable paper as a finished paper material. It is also possible to mix a binder in pulp slurry. In the wire part, wet paper is formed from the finished paper material supplied from the former in a paper making net. In the first dry part 17, the wet paper formed in the wire part is dried. In the spray part, the binder is sprayed onto the paper dried in the first dry part 17. In the second dry part 24, the paper in wet condition with the binder sprayed at the spray part is dried.

The finished paper material supplied from the former 14 is subjected to papermaking at the wire part, and wet paper is formed on the wire 15. Moisture in the wet paper is removed by suction by a suction box 16 installed at the wire part, so that the wet paper has a predetermined moisture content. The wet paper is then introduced into the first dry part 17 and dried. The first dry part 17 is configured with a through air dryer (hereinafter referred to as TAD). The TAD includes a rotating drum 18 whose circumferential surface is air permeable, and a hood 19 which covers the rotating drum 18 substantially airtightly. In the TAD, air heated to a predetermined temperature is supplied into the hood 19. The heated air flows from the outside to the inside of the rotating drum 18. The wet paper is conveyed while being held on the circumferential surface of the rotating drum 18 rotating in the arrow direction in FIG. 8. While being conveyed through the TAD, the heated air penetrates the wet paper in the thickness direction thereof, whereby the wet paper is dried and becomes paper.

At the spray part, an aqueous solution including a binder (water-soluble binder solution) is sprayed on the paper obtained at the first dry part 17. The spray part is at a position between the first and second dry parts 17, 24. Both dry parts 17, 24 are connected via a conveyor.

The conveyor is provided with an upper conveyor belt 20 and a lower conveyor belt 21 each rotating in the arrow direction. The conveyor 20 is configured to convey the paper dried by the TAD of the first dry part 17 to the second dry part 24 in a state of being sandwiched between these belts 20, 21. A vacuum roll 22 is arranged at a folding back end on the downstream side of the upper conveyor belt 20. The vacuum roll 22 attracts paper on the back surface of the upper conveyor belt 20, and conveys the upper conveyor belt 20 under the attracting state.

As shown in FIG. 8, the spray part is provided with a spray nozzle 23. The spray nozzle 23 is arranged below the second dry part 24, facing the vacuum roll 22. The spray nozzle 23 sprays a spray liquid including the binder toward the vacuum roll 22 and adds (externally adds) the spraying liquid to the paper.

After the binder is supplied at the spray part, the paper is conveyed to the second dry part 24. The second dry part 24 is configured with a Yankee dryer. The paper in a wet state by spraying the spraying liquid is conveyed while being held, on the circumferential surface of the rotating drum 25 of the Yankee dryer installed in the hood 26. The paper becomes dry while it is held and conveyed by the rotating drum 25.

The binder is supplied at the spray part at a position between the first and second dry parts 17 and 24. For example, the binder may be sprayed from above the upper conveyor belt 20 (the position indicated by the arrow between the first and second dry parts 17 and 24 shown in FIG. 8). Further, the binder may be sprayed from the upper side of the paper dried at the second dry part 24 (the position indicated by the arrow on the right side of the second dry part 24 shown in FIG. 8). Between the first and second dry parts 17, 24 and after the second dry part 24, the binder may be sprayed not only from the upper side but also from the lower side or from both the upper and lower sides.

In the present embodiment, in the papermaking step, the fiber orientation ratio in the length and width directions (length/width) of the base paper sheet is adjusted to 0.8 to 2.0, preferably 0.8 to 1.2. The fiber orientation can be adjusted in the papermaking machine, for example, by adjusting the angle at which the papermaking raw material is supplied to the wire part. The angle at which the papermaking raw material is supplied may be adjusted, for example, by adjusting the slice opening degree of the head box. Alternatively, the fiber orientation may be adjusted by giving vibration in a direction orthogonal to the conveyance direction (running direction) of the papermaking machine. [Ply Processing Step]

Next, the ply processing step (S2) of the present embodiment will be described. In the ply processing step (S2), as shown in FIG. 6, the continuous dry base paper 1A, 1A each continuously drawn out from the web roll 1 is supplied to an overlapping unit 2 for the ply process along the continuous direction to form a ply continuous sheet 1B. The overlapping unit 2 is configured with a pair of rolls, performs the ply process of each continuous dry base paper 1A, 1A to form a ply continuous sheet 1B to which the ply process has been applied. When overlapping the continuous dry base paper 1A, 1A, it may be weakly fastened with pin embosses (contact embosses) so that the continuous dry base paper 1A, 1A is not easily displaced.

[Solution Adding Step]

Next, the solution adding step (S3) of the present embodiment will be described. In the solution adding step (S3), as shown in FIG. 6, the water-soluble binder solution is sprayed on both outer surfaces (the surface of the continuous dry

## 11

base paper 1A, 1A which does not face the continuous dry base paper 1A, 1A after the ply process) of the ply continuous sheet (paper sheet) 1B by each of the two-fluid type spray nozzles 3, 3 to manufacture a continuous sheet 1C.

The water-soluble binder solution contains carboxyl methyl cellulose (CMC) as the water-soluble binder. In the water-soluble binder solution, and the blending ratio of CMC, to which cellulose nanofibers (CNF) are added, to CNF is preferably 9:1 to 1:1.

As a method of spraying the water-soluble binder solution, the water-soluble binder solution described above may be sprayed onto one of the outer surface of the ply continuous sheet 1B. A sheet equivalent to the continuous sheet 1C described above may be generated by spraying the above water-soluble binder solution from a two-fluid type spray nozzle on the outer surface (the surface of the sheet which does not face another sheet) of at least one of the continuous dry base paper 1A, 1A respectively drawn out from the above-described primary web rolls 1, 1, and immediately after that, by applying the ply process to the continuous dry base paper 1A, 1A.

The two-fluid type spray nozzle 3 is a spray nozzle for mixing and spraying compressed air and liquid divided into two systems. As compared with the one-fluid type spray nozzle from which sprays the compressed liquid alone, it is possible to spray the liquid finely and uniformly.

In the present embodiment, the nozzle diameter of the spray nozzle 3 is at most 0.09 gal/min. In addition, preferred spraying conditions of the present embodiment include the concentration of the water-soluble binder solution of 3.3 to 4.0%, the viscosity of the water-soluble binder solution of 900 to 3000 cPs, the discharge temperature of 50 to 70°C., the liquid pressure of 2 MPa or more, and the air pressure of 0.05 to 0.2 MPa.

By spraying the water-soluble binder solution onto the outer surface of the ply continuous sheet 1B in this way, the content of CMC and CNF in the toilet cleaning sheet gradually increases from the inside to the outside in the thickness direction. Therefore, it is possible to improve the surface strength while securing water-disintegrability, and to manufacture a toilet cleaning sheet with less damages even against strong rubbing.

The inside and outside in the thickness direction are determined as follows. In the case of application to both surfaces, the center part in the thickness direction is determined as the inside and the outer surface is determined as the outside. In the case of application to one surface, the surface to which the binder solution is not applied is determined as the inside, and the surface to which the binder solution is applied is determined as the outside.

## [Drying Step]

Next, the drying step (S4) of the present embodiment will be described. In the drying step (S4), as shown in FIG. 6, the insoluble liquid in the water-soluble binder solution of the continuous sheet 1C evaporates in the drying equipment 4, so that the effective ingredient, in particular CMC, is fixed to the fibers.

Here, since the amount of impregnated water-soluble binder solution decreases from the outside toward the inside in the thickness direction of the continuous sheet 1C, the CMC fixing amount decreases toward the inner side in the thickness direction. Therefore, in impregnation with the aqueous agent in the finishing step (S7) described later, the cross-linking reaction does not likely to occur and the number of gaps increases at the inner side in the thickness direction. As a result, the aqueous agent can be confined in the sheet. Therefore, the obtained toilet cleaning sheet is

## 12

difficult to dry. In addition, since a lot of CNF is present near the outside of the continuous sheet 1C in the thickness direction and a lot of cross-linking reaction of CMC occur near the outside of the continuous sheet 1C in the thickness direction, the surface strength of the obtained toilet cleaning sheet enhanced.

As the drying equipment 4, dryer equipment with a hood for blowing hot air against the continuous sheet 1C and drying it can be used. For more tight adhesion to each other, a press roll or a turn roll may be installed and the continuous sheet 1C may be passed through the press roll or the turn roll before the drying step (S4).

The drying equipment may be infra-red irradiation equipment. In this case, multiple infrared ray irradiation units are arranged in parallel in the conveyance direction of the continuous sheet 1C, and the continuous sheet 1C to be conveyed is irradiated with infrared rays and becomes dry. Since moisture is heated by the infrared rays and dried, it is can be uniformly dried compared with a dryer with hot air, and the occurrence of wrinkles in the slit-forming and winding step is prevented in the subsequent stage.

## [Slit-Forming and Winding Step]

Next, the slit-forming and winding step (S5) of the present embodiment will be described. In the slit-forming and winding step (S5), in order to prepare a web to be processed with an off-line processing machine from a continuous water-disintegrable sheet 1D to which the ply process has been applied, the continuous water-disintegrable sheet 1D dried in the drying step (S4) and to which CMC has been fixed is subjected to slit-formation at a predetermined width with a slitter 5 while adjusting the tension, and is wound in winder equipment 6. The winding speed is determined as appropriate considering the ply processing step (S2), solution adding step (S3) and drying step (S4). It should be noted that the sheet breaks if the winding speed is too rapid, and wrinkles will occur if it is too slow.

By crimping the continuous water-disintegrable sheet 1D to which the ply process has been applied in the slit-forming and winding step (S5), the continuous water-disintegrable sheet 1D is further integrated so as to be substantially one sheet.

## [Embossing Step]

Next, the embossing step (S6) of the present embodiment will be described. In the embossing step (S6), as shown in FIG. 7, the continuous water-disintegrable sheet 1D drawn out from the secondary web roll 11 is subjected to embossing for forming a predetermined shape on the entire surface of the sheet by the embossing roll 12. The object of this embossing is to enhance the strength, bulkiness, wiping property, etc. of the sheet and to improve the design.

## [Finishing Step]

Next, the finishing step (S7) of the present embodiment will be described. In the finishing step (S7), as shown in FIG. 7, the following steps are performed as a series of events in the finish processing equipment 13: cutting of the embossed sheet 1E; folding of the respective cut sheets, impregnation with the aqueous agent (including aqueous a detergent, a fragrance, an antiseptic, a disinfectant, a paper strengthening agent, organic solvent, etc.) to the respective folded sheets, and packaging of the respective sheets impregnated with the aqueous agent.

Through these steps, the toilet cleaning sheet is manufactured.

## EXAMPLES

Next, the result of wet tensile strength test will be described regarding Examples and Comparative Examples of the present invention.

## 13

CNF used here was CNF with 100% NBKP. CNF having an average fiber width (median diameter) of 49 nm was used. CNF was obtained by refiner treatment of NBKP for rough fibrillation, and treating it four times with a high pressure homogenizer for fibrillation.

Here, a method of measuring the fiber width (average fiber width) of CNF will be described.

First, 100 ml of an aqueous dispersion of cellulose nanofibers having a solid content concentration of 0.01 to 0.1 mass % is filtered with a Teflon (registered trademark) membrane filter, and the solvent is displaced once by 100 ml of ethanol and three times 20 ml by t-butanol.

Next, by freeze-drying and osmium-coating, a sample is obtained. This sample is observed in a SEM image by an electron microscope at a magnification of 5,000 times, 10,000 times, or 30,000 times (in the present embodiment, a magnification of 30,000 times) according to the width of the fibers constituting the sample. Specifically, two diagonal lines are drawn on the observed image, and arbitrarily three straight lines passing through the intersection of the diagonal lines are drawn. Further, the fiber width is visually measured from a total of 100 fibers which intersect with these three straight lines. Then, the median diameter of the measured values is taken as the average fiber diameter. The average fiber diameter is not limited to the median diameter of the measured value, but may be, for example, the number average diameter or the mode diameter (most frequent diameter).

The conditions for the respective Examples and Comparative Examples are described below.

The sample corresponding to the respective Examples and Comparative Examples was prepared as follows.

First, after the base paper having weighing (in a dry state) of 45 gsm was made to be two-ply in the water-soluble binder application equipment, an aqueous solution (water-soluble binder solution) including CMC and CNF mixed was applied to the outer surface of each sheet with a spray according to the following conditions.

At this time, the concentration of the aqueous solution was 3.0%, 3.3%, 3.5%, 3.8%, and 4.0%. The application amount on the sheet was adjusted depending on the concentration of the aqueous solution so that the total amount of CMC-CNF attached to the base paper sheet after the spray application was constant. Specifically, the application amount of the aqueous solution on the sheet was 40 gsm in wet application amount at the concentration of 3.0%, 36.4 gsm in wet application amount at the concentration of 3.3%, 34.3 gsm in wet application amount at the concentration of 3.5%, 31.6 gsm in wet application amount at the concentration of 3.8%, and 30 gsm in wet application amount at the concentration of 4.0%. The dry application amount was 1.2 gsm in all cases.

After that, the sheet was dried until the moisture percentage reached about 8% by passing through a hot air dryer (temperature 180° C.) and slits were formed at a predetermined width. A base sheet for processing the base paper sheet was thereby prepared. The sampled base paper sheet was uniformly impregnated with a chemical solution of 200% by weight of the weight of the sheet with a syringe and used as a sample.

## Example 1

Blend of pulp; NBKP:LBKP=40:60

Weighing (in a dry state); 90 g/m<sup>2</sup> (2-ply)

Item Number of CMC; CMC 1330 Daicel Corporation

CNF blending ratio; 10.0% by weight

## 14

Aqueous agent component; Cross-linking agent (zinc) 3.56% by weight, Propylene glycol monomethyl ether (PGME) 14.5% by weight, Propylene glycol (PG) 3.0% by weight

5 Impregnated amount of Aqueous agent; 200% by weight of base paper weight

Example 2

CNF blending ratio; 30.0% by weight

The other conditions are the same as in Example 1.

## Example 3

CNF blending ratio; 50.0% by weight

The other conditions are the same as in Example 1.

## Comparative Example 1

CNF blending ratio; 0.0% by weight

The other conditions are the same as in Example 1.

## Comparative Example 2

CNF blending ratio; 5.0% by weight

The other conditions are the same as in Example 1.

## Comparative Example 3

CNF blending ratio; 100.0% by weight

The other conditions are the same as in Example 1.

## 30 [Evaluation of Surface Strength]

<Test Method>

The samples corresponding to Examples 1 to 3 and Comparative Examples 1 to 3 were each cut off to width 75 mm×length 240 mm in the MD direction and in the CD direction without peeling off the ply, folded into three with both end regions in the width direction overlapped, and rubbed with a Gakushin type fastness rubbing tester at the portion to be measured. The number of rubbing was measured at the time when damage such as scuffing or tear was visually confirmed on the sheet. The measurement was performed three times for each of the MD direction and the CD direction, and the three measured values were averaged. The test conditions with the Gakushin type fastness rubbing tester were as follows.

45 Gakushin Type Fastness Rubbing Tester: manufactured by TESTER SANGYO CO., LTD., Item Number AB301

Rubbing Finger:

Shape 20 mm×R 50 mm

Load 200 gf (With white cotton cloth fixed, including arm)

Load Per Unit Area 50 gf/cm<sup>2</sup> (Load 200 gf/contact area 4.0 cm<sup>2</sup>)

50 As the fixed cotton cloth for the rubbing finger, one piece of PP band (Sekisui Jushi Corporation, Item Number 19K (width 15 mm×length 60 mm)) was fixed to the rubbing finger with screws so that there are no gaps or wrinkles.

Sample Holder:

|                         |         |
|-------------------------|---------|
| Shape                   | R200 mm |
| Stroke                  | 120 mm  |
| Reciprocating Frequency | 30 cps  |

60 65 Sample: Width 25 mm (A sample with a width of 75 mm was folded in three without peeling off the ply)×length 240 mm (Sample holder side)

## Test Procedure:

- (1) Mount the sample on the sample holder so that it is not loose.
- (2) Gently lower the rubbing finger to the sample holder.
- (3) Press the start SW to start the test.

Judgment Method: By confirming the state of the sample after Gakushin processing (rubbing), the number of rubbing was measured at the time when damage such as scuffing or tear was visually confirmed on the sheet.

In the above test, a PP band with a mesh pattern on the surface is used as the rubbing finger, assuming a case where the toilet cleaning sheet is actually used, that is, a case where the rim of a toilet bowl is rough due to attached stains. As a result, it is possible to conduct an environmental test assuming the actual use of the toilet cleaning sheet and to obtain highly reliable evaluation result on whether or not the toilet cleaning sheet is durable when actually used.

## &lt;Evaluation&gt;

FIG. 9 is a graph showing results of the above test in the MD direction. FIG. 10 is a graph showing results of the above test in the CD direction.

As shown in FIGS. 9 and 10, if the range of the concentration of the aqueous solution is at least 3.3% and at most 4.0% in Examples 1 to 3, the results exceeded the value (40 or more) as the criterion to determine whether or not the toilet cleaning sheet is durable when actually used. Therefore, it was found to be durable when actually used.

Further, according to Examples 1 to 3, it was found that if the concentration of the aqueous solution is in the range of at least 3.3% and at most 4.0%, the higher the concentration is, the more the measured value is.

On the other hand, in Comparative Examples 1 to 3, the results were below the value as a criterion. Therefore, it was found not to be durable when actually used.

## [Evaluation of Water-Disintegrability]

## &lt;Test Method&gt;

For samples corresponding to Examples 1 to 3 and Comparative Examples 1 to 3, the water-disintegrability was measured according to a method based on JIS P 4501 (2006) 4.5 "easiness of loosening".

## &lt;Evaluation&gt;

FIG. 11 is a graph showing results of the above test.

As shown in FIG. 11, in all of Examples 1 to 3, the results were about 40 seconds. Therefore, it was found that the water-disintegrability was good.

## [Evaluation of Viscosity]

## &lt;Test Method&gt;

Viscosity was measured using a single cylinder rotational viscometer (B-type viscometer) under conditions of 60°C. and 60 rpm for each of Examples 1 to 3 and Comparative Examples 1 to 3 with concentrations of the aqueous solution being 3.0%, 3.3%, 3.5%, and 4.0%.

TABLE 1 shows the results of the above test.

TABLE 1

| Concentration (%)     | 3.0  | 3.3  | 3.5  | 3.8  | 4.0  |
|-----------------------|------|------|------|------|------|
| Example 1             | 725  | 921  | 1154 | 1384 | 1564 |
| Example 2             | 1456 | 2721 | 3789 | 4124 | 4567 |
| Example 3             | 1989 | 3890 | 4890 | 5201 | 5679 |
| Comparative Example 1 | 330  | 419  | 550  | 661  | 797  |
| Comparative Example 2 | 456  | 514  | 656  | 789  | 925  |
| Comparative Example 3 | 3300 | 4190 | 5500 | 6610 | 7970 |

According to TABLE 1, if the range of the concentration of the aqueous solution is at least 3.3% and at most 4.0% in Examples 1 to 3, it is understood that the viscosity is at least 900 cPs.

Some of Examples 1 to 3 in TABLE 1 have viscosities of more than 3000 cPs, however, from the viewpoint of maintaining quality and handling during operations, the viscosity of the aqueous solution used for manufacture is preferably at most 3000 cPs.

As described above, according to the present embodiment, a water-soluble binder solution in which the blending ratio of CMC to CNF is 9:1 to 1:1 is used and the concentration thereof is set to be at least 3.3% and at most 4.0%.

10 As a result, the surface strength can be improved efficiently while water-disintegrability is maintained.

Accordingly, the surface strength can be improved without increasing the application amount of CMC in the water-soluble binder solution.

15 Although the present invention has been specifically described based on the embodiments, the present invention is not limited to the above-described embodiments, and modification can be made within a range not departing from the gist thereof.

20 For example, although a toilet cleaning sheet is described as an example of a water-disintegrable sheet in the embodiments of the present invention, the present invention is not limited thereto, and can be applied to products that are desired to be able to be thrown away after use with a large amount of water in toilet etc., such as a body wiping sheet for wiping the body and a sheet for wiping ass.

25 In describing the embodiments and the like of the present invention, the emboss EM11 with a protrusion PR21 having a curved shape and the emboss EM12 with a protrusion PR22 having a planar shape are shown as an example, but the emboss is not necessarily limited to these shapes, but may have any shape.

30 For example, in describing the embodiments and the like of the present invention, all of the embosses EM11 and EM12 project toward the front side of the drawing in FIG. 1. However, the embosses EM11 and EM12 projecting toward the front direction of the drawing and the embosses EM11 and EM12 recessed toward the front direction of the drawing may be arranged alternately.

35 Specifically, as shown in FIG. 12, by alternately arranging the embosses EM11 and EM12 projecting toward the front direction of the drawing in FIG. 12 (solid line portions) and the embosses EM11 and EM12 recessed toward the front direction of the drawing in FIG. 12 (broken line portions), it is possible to improve the surface strength of the water-disintegrable sheet and to provide a water-disintegrable sheet with high wiping property on either side of the toilet cleaning sheet 101 by the embosses.

40 FIGS. 13 to 15 show a modified example in which only the emboss pattern of the toilet cleaning sheet is different.

45 In FIGS. 13 to 15, the concave portion e2 has an inverted shape of the convex portion e1. The convex portion e1 and the concave portion e2 are alternately arranged in each of multiple rows. An emboss pattern is formed by arranging the multiple rows such that the convex portions e1 in adjacent rows are shifted from each other by a half pitch, and so are the concave portions e2. In this way, since the convex portions e1 and the concave portions e2 are alternately formed both in the length direction and the width direction, it is possible to improve the property of wiping stain compared with the emboss pattern in which the convex portions are arranged in a row or the concave portions are arranged in a row. The shapes of the convex portions e1 and the concave portions e2 are not particularly limited, and may be a circular shape, an elliptical shape, a polygonal shape, or the like. It may be a combination of the shapes.

17

In describing the embodiments and the like of the present invention, the water-soluble binder solution is applied with a spray, however, the binder solution may be applied to the continuous dry base paper 1A continuously drawn out from the first web roll 1 by a doctor chamber system (transfer equipment including two paired printing plate rolls with respect to one backup roll, anilox rolls paired with the respective printing plate rolls, and doctor chambers for applying the binder solution to the respective anilox rolls), and/or a three roll system (transfer equipment including two paired printing plate rolls with respect to one backup roll, anilox rolls paired with the respective printing plate rolls, dip rolls for applying the binder solution to the respective anilox rolls, and pans for applying the binder solution to the respective dip rolls). That is, in the solution adding step, from a printing machine(s) provided corresponding to at least one of the surfaces of the base paper serving as the front and back surfaces of the water-disintegrable sheet, the binder solution may be transferred to the corresponding base paper.

## INDUSTRIAL APPLICABILITY

The present invention is suitable for providing a water-disintegrable sheet such as a toilet cleaning sheet which is impregnated with an aqueous agent in advance, and a method for manufacturing the water-disintegrable sheet.

## REFERENCE SIGNS LIST

100, 101 Toilet Cleaning Sheet  
 1 Primary Web Roll  
 1A Continuous Dry Base Paper  
 1B Ply Continuous Sheet  
 1C Continuous Sheet  
 1D Continuous Water-Disintegrable Sheet  
 1E Embossed Sheet  
 2 Overlapping Unit  
 3 Spray Nozzle  
 4 First Drying Equipment  
 5 Slitter  
 6 Winder Equipment  
 11 Secondary Web Roll  
 12 Embossing Roll  
 13 Finish Processing Equipment  
 14 Former  
 15 Wire  
 16 Suction Box  
 17 first Dry Part  
 18 Rotating Drum  
 19 Hood  
 20 Upper Conveyor Belt  
 21 Lower Conveyor Belt  
 22 Vacuum Roll  
 23 Spray Nozzle  
 24 Second Dry Part  
 25 Rotating Drum  
 26 Hood  
 EM11, EM12, EM21 Emboss  
 PR21, PR22 Protrusion  
 HT21, HT22 Height Of Protrusion  
 CN31, SN32 Contact Area  
 e1 Convex Portion  
 e2 Concave Portion

The invention claimed is:

1. A water-disintegrable sheet comprising a base paper sheet, wherein:

18

the base paper sheet has a weight per unit area of 30 to 150 gsm,

the base paper sheet contains a water-soluble binder and cellulose nanofibers,

the base paper sheet is impregnated with an aqueous agent that includes a cross-linking agent which cross-links with the water-soluble binder,

in the base paper sheet, a content of the water-soluble binder and a content of the cellulose nanofibers gradually increase from inside toward outside of the base paper sheet in a thickness direction, and

when a wear resistance test is performed three times using a Gakushin type fastness rubbing tester with a PP band as a rubbing finger and an average of measured values for the three times is calculated for each of a MD direction and a CD direction, each average value is at least 40.

2. The water-disintegrable sheet according to claim 1, wherein:

the water-soluble binder has a carboxyl group, and the cross-linking agent is a metal ion.

3. The water-disintegrable sheet according to claim 1, wherein:

the water-soluble binder is carboxymethyl cellulose (CMC), and

the cross-linking agent is selected from the group consisting of alkaline earth metals, manganese, zinc, cobalt, and nickel.

4. The water-disintegrable sheet according to claim 1,

30 wherein the water-soluble binder and cellulose nanofibers are applied to at least one outer surface of the base paper sheet as a water-soluble binder solution containing the water-soluble binder and cellulose nanofibers.

5. The water-disintegrable sheet according to claim 1,

35 wherein the water-soluble binder and cellulose nanofibers are applied to two outer surface of the base paper sheet as a water-soluble binder solution containing the water-soluble binder and cellulose nanofibers.

6. The water-disintegrable sheet according to claim 1,

40 wherein:

the base paper sheet comprises a plurality of first embossed portions having a first shape and a plurality of second embossed portions having a second shape, the first shape being different from the second shape in a plan view of the base paper sheet,

45 the plurality of first embossed portions are arranged in a diamond lattice shape,

each of the plurality of second embossed portions is positioned between two of the first embossed portions,

50 wherein the first embossed portions are first protrusions, and the second embossed portions are second protrusions, and the first and second protrusions protrude in a same direction from a surface of the base paper sheet, and

55 wherein each of the second protrusions is continuous with two first protrusions adjacent thereto, to form a continuous embossed portion including both the first and second embossed portions.

7. The water-disintegrable sheet according to claim 1,

60 wherein:

the base paper sheet comprises a plurality of first embossed portions having a first shape and a plurality of second embossed portions having a second shape, the first shape being different from the second shape in a plan view of the base paper sheet,

65 the plurality of first embossed portions are arranged in a diamond lattice shape,

## 19

each of the plurality of second embossed portions is positioned between two of the first embossed portions, the plurality of the first embossed portions comprise a plurality of concave portions and a plurality of convex portions, all having the first shape, and the plurality of second embossed portions comprise a plurality of concave portions and a plurality of convex portions, all having the second shape.

8. The water-disintegrable sheet according to claim 1, wherein, in the base paper sheet, a ratio (length/width) of fiber orientation in length and width directions of the base paper sheet is 0.8 to 1.2.

9. A method for manufacturing a water-disintegrable sheet comprising:

applying a water-soluble binder solution including a water-soluble binder and cellulose nanofibers to an outer surface of a base paper sheet;  
 drying the sheet to which the water-soluble binder solution has been added; and  
 after the drying, applying an aqueous agent including a cross-linking agent which cross-links with the water-soluble binder to the sheet,  
 wherein a concentration of the water-soluble binder solution is at least 3.3%, the concentration of the water-soluble binder solution being a concentration of a total amount of the water-soluble binder and the cellulose nanofibers in the water-soluble binder solution,  
 wherein a blending ratio of the water-soluble binder to the cellulose nanofibers in the water-soluble binder solution is 9:1 to 1:1, and  
 wherein a viscosity of the water-soluble binder solution is at least 900 cP, when measured by a viscometer at 60° C. and 60 rpm.

10. The method according to claim 9, wherein the concentration of the water-soluble binder solution added in the addition of the solution is at least 3.5%.

## 20

11. The method according to claim 10, wherein the concentration of the water-soluble binder solution is at most 4.0%.

12. The method according to claim 9, wherein the concentration of the water-soluble binder solution is at most 4.0%.

13. The method according to claim 9, wherein the water-soluble binder solution is applied to both surfaces of the base paper sheet.

14. The method according to claim 9, wherein the water-soluble binder solution is applied to the base paper sheet while the base paper sheet is dry.

15. The method according to claim 9, wherein applying the binder solution comprises spraying the binder solution onto the outer surface of the base paper sheet.

16. The method according to claim 15, wherein the binder solution is sprayed onto the base paper sheet while the base paper sheet is dry.

17. The method according to claim 15, wherein the binder solution is sprayed onto both surfaces of the base paper sheet.

18. The method according to claim 9, wherein: the water-soluble binder

has a carboxyl group, and

the cross-linking agent is a metal ion.

19. The method according to claim 9, wherein:  
 the water-soluble binder is carboxymethyl cellulose (CMC), and

the cross-linking agent is selected from the group consisting of alkaline earth metals, manganese, zinc, cobalt, and nickel.

20. The method according to claim 9, wherein, in the base paper sheet, a ratio (length/width) of fiber orientation in length and width directions of the base paper sheet is 0.8 to 1.2.

\* \* \* \* \*